



US006090748A

# United States Patent [19]

Furuya et al.

[11] Patent Number: 6,090,748

[45] Date of Patent: Jul. 18, 2000

[54] **REVERSIBLE THERMOSENSITIVE RECORDING MATERIAL AND RECORDING METHOD AND RECORDING APPARATUS THEREFOR**

[75] Inventors: **Hiromi Furuya; Tadafumi Tatewaki**, both of Shizuoka-ken; **Masafumi Torii; Fumio Kawamura**, both of Shizuoka; **Hiroaki Matsui**, Numazu; **Masaru Shimada**, Shizuoka-ken; **Kyoji Tsutsui**, Mishima, all of Japan

[73] Assignee: **Ricoh Company, Ltd.**, Tokyo, Japan

[21] Appl. No.: **09/104,720**

[22] Filed: **Jun. 25, 1998**

[30] Foreign Application Priority Data

Jun. 26, 1997 [JP] Japan ..... 9-185917  
Jun. 26, 1997 [JP] Japan ..... 9-185918  
Jun. 24, 1998 [JP] Japan ..... 10-193769

[51] Int. Cl.<sup>7</sup> ..... **B41M 5/34**

[52] U.S. Cl. ..... **503/201**; 347/179; 503/209; 503/216; 503/217; 503/220; 503/221

[58] Field of Search ..... 503/200, 201, 503/216, 217, 221, 226, 220, 205, 208, 209; 347/179

[56] References Cited

U.S. PATENT DOCUMENTS

5,143,893 9/1992 Mochizuki et al. ..... 503/227  
5,229,189 7/1993 Hiyoshi et al. ..... 428/195  
5,250,346 10/1993 Nagai et al. ..... 428/195  
5,306,687 4/1994 Furuya et al. ..... 503/207  
5,380,693 1/1995 Goto ..... 503/200  
5,403,810 4/1995 Sawamura et al. ..... 503/201  
5,447,900 9/1995 Suzaki et al. ..... 503/207  
5,472,931 12/1995 Morohoshi ..... 503/227  
5,482,912 1/1996 Furuya et al. ..... 503/207  
5,489,501 2/1996 Torii et al. ..... 430/341  
5,521,138 5/1996 Shimada et al. ..... 503/209  
5,532,201 7/1996 Goto ..... 503/213  
5,547,500 8/1996 Tsutsui ..... 106/21 A

5,622,909 4/1997 Furuya et al. ..... 503/216  
5,641,724 6/1997 Yamaguchi et al. ..... 503/221  
5,679,615 10/1997 Matsumoto et al. ..... 503/217  
5,703,005 12/1997 Torii et al. ..... 503/201  
5,817,599 10/1998 Iida et al. ..... 503/209

FOREIGN PATENT DOCUMENTS

2135466 8/1984 United Kingdom .  
2320582 6/1998 United Kingdom .  
9622885 of 1996 WIPO ..... 503/201

OTHER PUBLICATIONS

WPI Acc No.: 97-53758, Abstract of JP 090254545A (Sep. 1997) (Mitsubishi, Mar. 1996).  
WPI Acc No.: 95-127979, Abstract of JP 070052553A (Feb. 1995) (Mitsubishi, Aug. 1993).  
WPI Acc No.: 95-125933, Abstract of JP 070047766A (Feb. 1995) (Mitsubishi, Aug. 1993).  
WPI Acc No.: 97-149289, Abstract of JP090024670A (Jan. 1997) (Ricoh), Jul. 1995).  
WPI Acc No.: 96-338205, Abstract of JP080156410A (Jun. 1996) (Mitsubishi, Dec. 1994).

Primary Examiner—Bruce H. Hess  
Attorney, Agent, or Firm—Cooper & Dunham LLP

[57]

ABSTRACT

A reversible thermosensitive recording material which includes a recording layer including an electron donating coloring agent and an electron accepting coloring developer and in which an image is reversibly formed and erased by appropriately heating and cooling the recording layer, wherein the recording material has an image density retention not less than about 60% when the recording material having an image is allowed to settle in a dry place at 50° C. for 24 hours, a residual image density not greater than about 0.03 when the recording material having an image is heated at 110° C. for 0.5 seconds to erase the image, and a residual image density after light irradiation not greater than about 0.04 when the recording material having an image is heated at 110° C. for 0.5 seconds to erase the image after light of 5,000 lux is irradiated to the recording material for 100 hours.

15 Claims, 1 Drawing Sheet



Fig. 1



## 1

**REVERSIBLE THERMOSENSITIVE  
RECORDING MATERIAL AND RECORDING  
METHOD AND RECORDING APPARATUS  
THEREFOR**

**BACKGROUND OF THE INVENTION**

1. Field of the Invention

The present invention relates to a reversible thermosensitive recording material, and a recording method and a recording apparatus therefor, and more particularly to a reversible thermosensitive recording material which utilizes a coloring reaction of an electron donating coloring agent and an electron accepting coloring developer and in which a colored image is repeatedly formed and erased by appropriately heating and cooling the reversible thermosensitive recording material, and a recording method and a recording apparatus therefor.

2. Discussion of the Related Art

A variety of thermosensitive recording materials are well known in which a colored image can be formed by a coloring reaction when an electron donating coloring agent is brought into contact with an electron accepting coloring developer while heat or the like is applied thereto.

The thermosensitive recording materials have the following advantages over other conventional recording materials:

- (1) color images can be rapidly recorded by a relatively simple apparatus without using such complicated steps as developing and fixing;
- (2) color images can be recorded without producing noise and environmental pollution;
- (3) various color images, e.g., red, blue, violet and black, can be easily obtained;
- (4) image density and background whiteness are high; and
- (5) the manufacturing cost is relatively low.

Because of these advantages, the above-described thermosensitive recording materials can be widely used, not only as a recording material for price labels in stores, but also as recording materials for copiers, printers for computers, facsimiles, automatic vending machines of tickets, video printers and measuring instruments.

However, the coloring reaction of these thermosensitive recording materials is irreversible and accordingly these recording materials cannot be repeatedly used.

Several thermosensitive recording materials which can reversibly form and erase an image have been proposed. For example, they are as follows:

- (1) a thermosensitive recording material which includes gallic acid in combination with phloroglucinol serving as coloring developers (Japanese Laid-Open Patent Publication No. 60-193691);
- (2) a thermosensitive recording material which includes phenolphthalein or Thymolphthalein serving as a coloring developer (Japanese Laid-Open Patent Publication No. 61-237684);
- (3) a thermosensitive recording material which includes an uniform solid solution of a coloring agent, a coloring developer and a carboxylic acid ester (Japanese Laid-Open Patent Publications No. 62-138556, 62-138568 and 62-140881);
- (4) a thermosensitive recording material which includes an ascorbic acid derivative serving as a coloring developer (Japanese Laid-Open Patent Publication No. 63-173684); and
- (5) a thermosensitive recording material which includes bis (hydroxyphenyl) acetic acid or a higher aliphatic amine salt of gallic acid serving as a coloring developer (Japanese Laid-Open Patent Publication No. 2-188294).

## 2

Some of the present inventors, jointly with others, have proposed a reversible thermosensitive coloring composition which includes a coloring agent such as a leuco dye and a coloring developer such as an organic phosphate compound,

- 5 an aliphatic carboxylic acid compound or a phenolic compound each of which has a long-chain aliphatic hydrocarbon group, and a reversible thermosensitive recording material using the coloring composition (Japanese Laid-Open Patent Publication No. 5-124360). The reversible thermosensitive recording material can stably repeat image formation and image erasure by being appropriately heated and cooled, and the image-recorded state or the image-erased state can be stably maintained at room temperature. In addition, Japanese Laid-Open Patent Publication No. 6-210954 has disclosed a
- 10 reversible thermosensitive recording material which includes a specified phenolic compound having a long-chain aliphatic hydrocarbon group serving as a coloring developer.

Thus reversible thermosensitive recording materials have been proposed; however, these recording materials do not have requisite properties of quick erasability and good preservability when they are used under various environmental conditions of temperature and humidity or when light is irradiated thereto. In attempting to improve the preservability, Japanese Laid-Open Patent Publications No. 7-164746 and 7-179043 have disclosed reversible thermosensitive recording materials which include a specified phenolic compound as a coloring developer. However, these recording materials cannot improve the preservability because an image recorded in the recording material cannot be clearly erased when the image is erased after light of 5000 lux is irradiated to the image for 100 hours. When these recording materials are in practical use in the market, a serious problem may occur in which information recorded in the recording materials is misunderstood.

In addition, these reversible thermosensitive recording materials have a drawback in that the image density deteriorates or the recording layer becomes deformed when images are repeatedly formed and erased in various environmental conditions of practical use of the recording materials (a problem hereinafter termed "deformation"). The reason for the deformation is considered to be that the structures of the recording layer and the protective layer of the recording material are gradually changed and deteriorated by the mechanical force and the heat of a thermal printhead which applies heat to the recording material to form or erase images.

In attempting to solve this problem, a reversible thermosensitive recording material has been disclosed which has a recording layer including particles whose average particle diameter is more than 1.1 times the thickness of the recording layer (Japanese Laid-Open Patent Publication No. 6-340171). In addition, a reversible thermosensitive recording material has been disclosed which has good ability to be used with thermal printheads owing to the formation of a protective layer thereon which has specified gloss and surface smoothness (Japanese Laid-Open Patent Publication No. 8-156410). However, these recording materials cannot yet entirely prevent the deterioration of the recording layer and the protective layer, which results in occurrence of deformation of the recorded image when the recording materials are repeatedly used. Therefore, these recording materials have a short life.

Further, Japanese Laid-Open Patent Publication No. 8-132738 has disclosed a reversible thermosensitive recording material which includes a compound selected from the group consisting of amide compounds, ester compounds, urea compounds and ketone compounds together with a dye

having a lactone ring which serves as a coloring agent, an irreversible coloring developer having a phenolic hydroxy group and a resin having color erasability. This recording material is different from the reversible thermosensitive recording material which utilizes a coloring/decolorizing reaction of a coloring agent and a coloring developer and to which the present invention relates. In addition, this recording material has a drawback in that it takes a long time (about 30 seconds) to erase an image and therefore rapid image erasure is difficult when using the recording material.

Because of these reasons, a need exists for a reversible thermosensitive recording material which has such good image formation/erasure ability, good preservability, and good durability as to be able to be repeatedly used in market for a long time.

#### SUMMARY OF THE INVENTION

Accordingly, an object of the present invention is to provide a reversible thermosensitive recording material which has good image formation/erasure ability even when the recording material is repeatedly used under various environmental conditions of practical use.

Another object of the present invention is to provide a reversible thermosensitive recording material having quick erasability, good preservability and good durability without occurrence of deformation of the recording material.

The invention also embraces a recording method and a recording apparatus using such a reversible thermosensitive recording material.

To achieve such objects, the present invention contemplates the provision of a reversible thermosensitive recording material which includes a recording layer including a reversible thermosensitive coloring composition including an electron donating coloring agent and an electron accepting coloring developer and in which an image is reversibly formed and erased by appropriately heating and cooling the recording layer, wherein the recording material has preservability such that an image density retention of a recorded image is not less than about 60% when the image is preserved in a dry place at 50° C. for 24 hours, quick erasability such that an residual image density of an image is not greater than about 0.03 when the image is erased at 110° C. for 0.5 seconds, and erasability after light irradiation in which an residual image density of an image is not greater than 0.04 when the image is erased at 110° C. for 0.5 seconds after light of 5000 lux is irradiated to the image for 100 hours.

The recording layer includes at least one color formation/erasure controlling agent having a formula selected from the group consisting of the following formulas (1) and (2):



wherein X1 represents a group including  $-CO-$ ,  $-NH-$  or  $-O-$ ; X2 represents a divalent group including  $-CO-$ ,  $-NH-$  or  $-O-$ ; R1 represents a divalent hydrocarbon group having carbon atoms of from 2 to 20, and when X1 is a carboxyl group, the R1 group adjacent to X1 is a linear hydrocarbon group having seven or more carbon atoms; R2 represents a hydrocarbon group having from 1 to 22 carbon atoms; and n is an integer of from 1 to 4, and when n is 2 or greater, each of R1 may be the same or different from each other and each of X2 may be the same or different from each other, and



wherein Y1 and Y2 independently represent a divalent group including  $-CO-$ ,  $-NH-$  or  $-O-$ ; R1 represents a divalent hydrocarbon group having from 2 to 20 carbon atoms; each of R2 and R2', independently represents a hydrocarbon group having from 1 to 22 carbon atoms; and n is 0 or an integer of from 1 to 4, and when n is 2 or greater, each of R1 may be the same or different from each other and each of Y2 may be the same or different from each other.

In another embodiment of the present invention, a reversible thermosensitive recording method for the reversible thermosensitive recording material is provided, including the steps of recording by imagewise heating the recording layer of the recording material of the present invention at a temperature not lower than an image forming temperature to form a colored image in the recording material and erasing by heating the colored image at a temperature lower than the image forming temperature and not lower than an image erasing temperature.

In yet another embodiment of the present invention, a reversible thermosensitive recording apparatus for the reversible thermosensitive recording material is provided which includes an image forming device which imagewise heats the recording layer of the recording material at a temperature not lower than an image forming temperature to form an image in the recording layer when the recording layer is cooled, and an image erasing device which heats the recording layer at a temperature lower than the image forming temperature and not lower than an image erasing temperature to erase the image, wherein the image erasing device is selected from the group consisting of ceramic heaters, plane heaters, heat rollers, heat bars and thermal printheads.

These and other objects, features and advantages of the present invention will become apparent upon consideration of the following description of the preferred embodiments of the present invention taken in conjunction with the accompanying drawing.

#### BRIEF DESCRIPTION OF THE DRAWING

FIG. 1 is a graph illustrating the relationship between temperature and image density of a recording layer in an image recording and erasing cycle of a reversible thermosensitive recording material embodying the present invention.

#### DESCRIPTION OF THE PREFERRED EMBODIMENTS

FIG. 1 is a graph illustrating the relationship between temperature of a reversible thermosensitive recording material (hereinafter a recording material) and image density thereof. When the recording material which is in a non-colored state A is heated, the recording material begins to color at an image forming temperature T1 in which at least one of an electron donating coloring agent and an electron accepting coloring developer is melted and then achieves a melted colored state B. If the recording material in the melted colored state B is rapidly cooled to room temperature, the recording material keeps the colored state and achieves a cooled colored state C in which the electron donating coloring agent and the electron accepting coloring developer are almost solidified. It depends upon cooling speed whether the recording material remains in the colored state, and if the recording material is gradually cooled, the recording material returns to the non-colored state A (a

dotted line B-A) or achieves a semi-colored state in which the image density of the recording material is relatively low compared to the image density of the recording material in the cooled colored state C. If the recording material in the cooled colored state C is heated again, the recording material begins to discolor at an image erasing temperature T2 lower than T1 and achieves a non-colored state E (a broken line C-D-E). If the recording material in the non-colored state E is cooled to room temperature, the recording material returns to the non-colored state A. The temperatures T1 and T2 depend on the materials of the coloring agent and the coloring developer. Accordingly, by appropriately selecting a coloring agent and a coloring developer, a recording material having desired T1 and T2 can be obtained. The image densities of the recording material in the colored states B and C are not necessarily the same.

In the colored state C, the recording layer includes the coloring agent and the coloring developer which form a solid in which a molecule of the coloring agent and a molecule of the coloring developer are mixed while contacting with each other. Namely, the coloring agent and the coloring developer cohere while they are reacting with each other, resulting in maintenance of the colored state. It is considered that the colored state C is stable because the semi-stable cohered structure of the coloring agent and the coloring developer is formed. On the other hand, in the non-colored state, at least one of the coloring agent and the coloring developer aggregates to form a domain, or crystallizes; thereby each phase of the coloring agent and the coloring developer which has a stable adhered structure is isolated from the other, and accordingly the recording material is stably in the non-colored state. In the recording materials of the present invention, the cohered structure of the coloring agent and the coloring developer is changed to a state in which the phases of the coloring agent and the coloring developer are isolated from the other and the coloring developer crystallizes; thereby color erasure can be perfectly performed. Namely, in the color erasure process of going from the colored state B to the non-colored state A when the recording materials are gradually cooled or going from the colored state C to the non-colored state A via the states D and E in FIG. 1, this structure change occurs at the image erasing temperature T2. The more stable the semi-stable cohered structure and the stable cohered structure of a recording material, the better the preservability of formed images and the erasability of the recording material.

The residual image density which means optical density of an erased image mainly depends on structure change of coloring agents. The present inventors have discovered that structure changes such as oxidation of coloring agents can be prevented by using a specified phenolic compound as a coloring developer and thereby a recording material having good erasability can be obtained. In addition, it is discovered that a recording material having good preservability (particularly at high temperature) and good erasability can be obtained by including a specified color formation/erasure controlling agent in the recording layer. The reason for the resultant improvement of the preservability is considered to be as follows:

- (1) in a colored state of the recording material, the color formation/erasure controlling agent comes to be included in the cohered structure of the coloring agent and the coloring developer; and thereby a more stable cohered structure can be formed; and
- (2) in a non-colored state, the color formation/erasure controlling agent that has a strong cohered structure accelerates the crystallization of the coloring developer; and thereby images can be clearly erased.

The reversible thermosensitive recording material of the present invention has a substrate, a recording layer formed

on the substrate and optionally a protective layer formed on the recording layer. The structure of the recording material of the present invention need not be limited to this structure. For example, the recording material may include an under-coat layer formed between the substrate and the recording layer, an intermediate layer formed between the recording layer and the protective layer, and a back-coat layer formed on the side of the substrate opposite to the side on which the recording layer is formed. In addition, the recording material may include a magnetic recording layer.

The present invention provides a reversible thermosensitive recording material which includes a recording layer including a reversible thermosensitive coloring composition including an electron donating coloring agent and an electron accepting coloring developer and optionally a resin and in which an image is reversibly formed and erased by appropriately heating and cooling the recording layer, wherein the recording material has preservability such that an image density retention of an image is not less than about 60% and preferably not less than about 70% when the image is preserved in a dry place (not greater than 40% RH and not greater than 30% RH as a severe condition) at 50°C. for 24 hours, quick erasability such that an residual image density is not greater than about 0.03 and preferably not greater than about 0.02 when an image is erased at 110°C. for 0.5 seconds, and erasability after light irradiation such that an residual image density is not greater than about 0.04 and preferably not greater than about 0.03 when an image is erased at 110°C. for 0.5 seconds after light of 5000 lux is irradiated to the image for 100 hours.

The image density retention is defined as follows:

$$\text{Image density retention (\%)} = \frac{(ID_2 - GD_2)}{(ID_1 - GD_1)} \times 100$$

wherein ID1 and ID2 represent image density of an image before and after the recording material having the image is preserved at 50°C. for 24 hours, respectively, and GD1 and GD2 represent background density of the image before and after the recording material having the image is preserved at 50°C. for 24 hours, respectively. The image density and background density can be measured with a conventional densitometer such as a reflection densitometer or a transmittance densitometer which is used for measuring the image density of an image formed on a transparent recording material.

The residual image density is defined as follows:

$$\text{Residual image density} = ID_r - GD$$

wherein IDr represents a reflection (or transmittance) density of a portion of a recording material in which an image has been recorded and then erased, and GD represents a background density of the recorded image in the recording layer. The densities IDr and GD can be also measured with the densitometer mentioned above.

To obtain good preservability and quick erasability, the recording layer of the present invention includes at least one color formation/erasure controlling agent having a formula selected from the group consisting of the following formulas (1) and (2):



wherein X1 represents a group including at least one of groups, —CO—, —NH— and —O—; X2 represents a divalent group including at least one of groups, —CO—,

—NH— and —O—; R1 represents a divalent hydrocarbon group having from 2 to 20 carbon atoms, and when X1 is a carboxyl group, the R1 group adjacent to X1 is a linear hydrocarbon group having seven or more carbon atoms; R2 represents a hydrocarbon group having from 1 to 22 carbon atoms; and n is an integer of from 1 to 4, and when n is 2 or greater, each of R1 may be the same or different from each other and each of X2 may be the same or different from each other; and



wherein Y1 and Y2 independently represent a divalent group including at least one of groups, —CO—, —NH— and —O—; R1 represents a divalent hydrocarbon group having from 2 to 20 carbon atoms; R2 and R2' independently represents a hydrocarbon group having from 1 to 22 carbon

atoms; and n is 0 or an integer of from 1 to 4, and when n is 2 or greater, each of R1 may be the same or different from each other and each of Y2 may be the same or different from each other.

R1, R2 and R2' are optionally substituted with a hydroxide group, a halogen atom, an alkoxy group or the like. In addition, any one or more of R1, R2 and R2' may be an aliphatic hydrocarbon group or an aromatic hydrocarbon group, or a hydrocarbon group in which an aliphatic hydrocarbon group and an aromatic hydrocarbon group are combined. Further, the aliphatic hydrocarbon group may be linear or branched, and may include an unsaturated bonding.

The total carbon number (number of carbon atoms) of R1, R2 and R2' is preferably not less than 8, and more preferably not less than 11, to maintain good image formation/erasure properties.

Suitable groups for use as R1 include groups shown in Table 1.

TABLE 1



wherein q, q', q'' and q''' are independently an integer not greater than the carbon number of R1 which is determined depending on the carbon numbers of R2 and R2', and the total carbon number in a group is not greater than the carbon number of R1.

Suitable groups for use as R2 or R2' include the groups shown in Table 2.

TABLE 2



wherein q, q', q" and q''' are independently an integer not greater than the carbon number of R2 or R2' each of which is determined depending on the carbon numbers of R1 and R2' or R1 and R2, and the total carbon number in a group is not greater than the carbon number of R2 or R2'.

Suitable groups for use as X1 include the groups having at least one of groups, —NH—, —CO—, and —O—.

Specific examples of X1 include groups shown in Table 3.

TABLE 3



45 Suitable groups for use as X2, Y1 and Y2 include divalent groups having at least one of groups, —NH—, —CO—, and —O—.

Specific examples of X2, Y1 and Y2 include groups shown in Table 4.

TABLE 4



TABLE 4-continued



In the color formation/erasure controlling agents for use in the present invention, a compound having either one of the following formulas (9) and (10) has a color developing ability; however, it is observed that when the carbon number of R1 of the compound is 7 or more, the color developing ability thereof decreases and the color formation/erasure ability increases.



Suitable color formation/erasure controlling agents include compounds having the following formulas (11) to (14), but are not limited thereto:



wherein R1' and X2' independently represent one of the groups which are mentioned above for use as R1 and X2, and when n is 2 or more, each of R1' may be the same or different from each other and each of X2' may be the same or different from each other.

More suitable compounds for use as color formation/erasure controlling agents include compounds having the following formulas (15) to (18):



wherein a and a' are independently an integer of from 2 to 20, and m and m' are independently an integer of from 1 to 22.

Specific examples of such compounds having formula (15) include compounds shown in Table 5.

TABLE 5



In addition, specific examples of such compounds having formula (16) include compounds similar to those shown in Table 5.

More specifically, examples of the compound having the formula,  $\text{HO}-(\text{CH}_2)_a-\text{NHCONH}-(\text{CH}_2)_{m-1}-\text{CH}_3$ , which is shown in Table 5 include compounds shown in Table 6.

TABLE 6

$\text{HO}-(\text{CH}_2)_2-\text{NHCONH}-(\text{CH}_2)_{17}\text{CH}_3$   
 $\text{HO}-(\text{CH}_2)_3-\text{NHCONH}-(\text{CH}_2)_{17}\text{CH}_3$   
 $\text{HO}-(\text{CH}_2)_5-\text{NHCONH}-(\text{CH}_2)_{17}\text{CH}_3$   
 $\text{HO}-(\text{CH}_2)_7-\text{NHCONH}-(\text{CH}_2)_{17}\text{CH}_3$   
 $\text{HO}-(\text{CH}_2)_9-\text{NHCONH}-(\text{CH}_2)_{17}\text{CH}_3$   
 $\text{HO}-(\text{CH}_2)_{11}-\text{NHCONH}-(\text{CH}_2)_{17}\text{CH}_3$   
 $\text{HO}-(\text{CH}_2)_{12}-\text{NHCONH}-(\text{CH}_2)_{17}\text{CH}_3$   
 $\text{HO}-(\text{CH}_2)_5-\text{NHCONH}-(\text{CH}_2)_{21}\text{CH}_3$   
 $\text{HO}-(\text{CH}_2)_5-\text{NHCONH}-(\text{CH}_2)_{20}\text{CH}_3$   
 $\text{HO}-(\text{CH}_2)_5-\text{NHCONH}-(\text{CH}_2)_{19}\text{CH}_3$   
 $\text{HO}-(\text{CH}_2)_5-\text{NHCONH}-(\text{CH}_2)_{14}\text{CH}_3$   
 $\text{HO}-(\text{CH}_2)_{11}-\text{NHCONH}-(\text{CH}_2)_{21}\text{CH}_3$   
 $\text{HO}-(\text{CH}_2)_{11}-\text{NHCONH}-(\text{CH}_2)_{14}\text{CH}_3$   
 $\text{HO}-(\text{CH}_2)_{11}-\text{NHCONH}-(\text{CH}_2)_6\text{CH}_3$   
 $\text{HO}-(\text{CH}_2)_{14}-\text{NHCONH}-(\text{CH}_2)_2\text{CH}_3$   
 $\text{HO}-(\text{CH}_2)_{17}-\text{NHCONH}-\text{CH}_3$

Specific examples of such compounds having formula (17) include compounds shown in Table 7.

TABLE 7

In addition, specific examples of such compounds having formula (18) include compounds similar to those shown in Table 7.

More specifically, examples of the compounds having the formula,  $\text{CH}_3(\text{CH}_2)_{m'-1}-\text{NHCONH}-(\text{CH}_2)_{m-1}\text{CH}_3$ , or  $\text{CH}_3(\text{CH}_2)_{m'-1}-\text{NHCONH}-(\text{CH}_2)_a-\text{NHCONH}-(\text{CH}_2)_{m'-1}\text{CH}_3$ , which are shown in Table 7 include compounds shown in Table 8.

TABLE 8

$$\begin{aligned}
 & \text{CH}_3(\text{CH}_2)_{17}\text{—NHCONH—}(\text{CH}_2)_{17}\text{CH}_3 \\
 & \text{CH}_3(\text{CH}_2)_{17}\text{—NHCONH—CH}_3 \\
 & \text{CH}_3(\text{CH}_2)_{17}\text{—NHCONH—}(\text{CH}_2)_5\text{CH}_3 \\
 & \text{CH}_3(\text{CH}_2)_{17}\text{—NHCONH—}(\text{CH}_2)_{11}\text{CH}_3 \\
 & \text{CH}_3(\text{CH}_2)_{17}\text{—NHCONH—}(\text{CH}_2)_{14}\text{CH}_3 \\
 & \text{CH}_3(\text{CH}_2)_{17}\text{—NHCONH—}(\text{CH}_2)_{21}\text{CH}_3 \\
 & \text{CH}_3(\text{CH}_2)_{7}\text{—NHCONH—CH}_2\text{CH}_3 \\
 & \text{CH}_3(\text{CH}_2)_{7}\text{—NHCONH—}(\text{CH}_2)_5\text{CH}_3 \\
 & \text{CH}_3(\text{CH}_2)_{21}\text{—NHCONH—}(\text{CH}_2)_5\text{CH}_3
 \end{aligned}$$

TABLE 8-continued

The content of the color formation/erasure controlling agent in the recording layer is preferably from about 0.1 to about 300% by weight, and more preferably from about 3 to 100% by weight, of the coloring developer in the recording

The recording layer of the reversible thermosensitive recording material of the present invention preferably includes one of leuco dyes having the following formulas (3), (5) and (6) which serve as an electron donating compound, to obtain good color forming ability.



wherein R3 and R4 independently represent a lower alkyl group, an aryl group which is optionally substituted, or a hydrogen atom, and R3 and R4 may combine with each other to form a ring; R5 represents a lower alkyl group, a halogen atom or a hydrogen atom; and R6 represents a lower alkyl group, a halogen atom, a hydrogen atom or a substituted anilino group having the following formula (4),



65 wherein R7 represents a lower alkyl group or a hydrogen atom; and X3 represents a lower alkyl group or a halogen atom; and b is 0 or an integer of from 1 to 3;

15



wherein R8–R11 independently represent an alkyl group or a hydrogen atom; and R12 represents an alkyl group, an alkoxy group or a hydrogen atom; and



wherein R13–R16 independently represent a lower alkyl group or a hydrogen atom; and R17 and R18 independently represent an alkyl group, an alkoxy group or a hydrogen atom.

Specific examples of leuco dyes for use as a coloring agent in the recording layer of the recording material of the present invention include, but are not limited to:

- 2-anilino-3-methyl-6-diethylaminofluoran,  
 2-anilino-3-methyl-6-(di-n-butylamino)fluoran,  
 2-anilino-3-methyl-6-(N-n-propyl-N-methylamino) 40  
 fluoran,  
 2-anilino-3-methyl-6-(N-isopropyl-N-methylamino)  
 fluoran,  
 2-anilino-3-methyl-6-(N-isobutyl-N-methylamino) 45  
 fluoran,  
 2-anilino-3-methyl-6-(N-n-amyl-N-methylamino)  
 fluoran,  
 2-anilino-3-methyl-6-(N-sec-butyl-N-methylamino) 50  
 fluoran,  
 2-anilino-3-methyl-6-(N-n-amyl-N-ethylamino)fluoran,  
 2-anilino-3-methyl-6-(N-n-isoamyl-N-ethylamino) 55  
 fluoran,  
 2-anilino-3-methyl-6-(N-n-propyl-N-isopropylamino)  
 fluoran,  
 2-anilino-3-methyl-6-(N-cyclohexyl-N-methylamino) 60  
 fluoran,  
 2-anilino-3-methyl-6-(N-ethyl-p-toluidino)fluoran,  
 2-anilino-3-methyl-6-(N-methyl-p-toluidino)fluoran,  
 2-(m-trichloromethylanilino)-3-methyl-6- 65  
 diethylaminofluoran,  
 2-(m-trifluoromethylanilino)-3-methyl-6-  
 diethylaminofluoran,  
 2-(m-trichloromethylanilino)-3-methyl-6-(N-cyclohexyl-  
 N-methylamino)fluoran,
- 16
- 2-(2,4-dimethylanilino)-3-methyl-6-diethylaminofluoran,  
 2-(N-ethyl-p-toluidino)-3-methyl-6-(N-ethylanilino) 5  
 fluoran,  
 2-(N-ethyl-p-toluidino)-3-methyl-6-(N-propyl-p-  
 toluidino)fluoran,  
 2-anilino-6-(N-n-hexyl-N-ethylamino)fluoran,  
 2-(o-chloroanilino)-6-diethylaminofluoran,  
 2-(o-chloroanilino)-6-dibutylaminofluoran,  
 2-(m-trifluoromethylanilino)-6-diethylaminofluoran,  
 2,3-dimethyl-6-dimethylaminofluoran,  
 3-methyl-6-(N-ethyl-p-toluidino)fluoran,  
 2-chloro-6-diethylaminofluoran,  
 2-bromo-6-diethylaminofluoran,  
 2-chloro-6-dipropylaminofluoran,  
 3-chloro-6-cyclohexylaminofluoran,  
 3-bromo-6-cyclohexylaminofluoran,  
 2-chloro-6-(N-ethyl-N-isoamylamino)fluoran,  
 2-chloro-3-methyl-6-diethylaminofluoran,  
 2-anilino-3-chloro-6-diethylaminofluoran,  
 2-(o-chloroanilino)-3-chloro-6-cyclohexylaminofluoran,  
 2-(m-trifluoromethylanilino)-3-chloro-6- 25  
 diethylaminofluoran,  
 2-(2,3-dichloroanilino)-3-chloro-6-diethylaminofluoran,  
 1,2-benzo-6-diethylaminofluoran,  
 3-diethylamino-6-(m-trifluoromethylanilino)fluoran,  
 3-(1-ethyl-2-methylindole-3-yl)-3-(2-ethoxy-4- 30  
 diethylaminophenyl)-4-azaphthalide,  
 3-(1-octyl-2-methylindole-3-yl)-3-(2-ethoxy-4-  
 diethylaminophenyl)-4-azaphthalide,  
 3-(1-ethyl-2-methylindole-3-yl)-3-(2-ethoxy-4-  
 diethylaminophenyl)-7-azaphthalide,  
 3-(1-ethyl-2-methylindole-3-yl)-3-(2-methyl-4-  
 diethylaminophenyl)-4-azaphthalide,  
 3-(1-ethyl-2-methylindole-3-yl)-3-(2-methyl-4-  
 diethylaminophenyl)-7-azaphthalide,  
 3-(1-ethyl-2-methylindole-3-yl)-3-(4-N-n-amyl-N- 35  
 methylaminophenyl)-4-azaphthalide,  
 3-(1-methyl-2-methylindole-3-yl)-3-(2-hexyloxy-4-  
 diethylaminophenyl)-4-azaphthalide,  
 3,3-bis(2-ethoxy-4-diethylaminophenyl)-4-azaphthalide,  
 and  
 3,3-bis(2-ethoxy-4-diethylaminophenyl)-7-azaphthalide.
- The coloring agent for use in the recording layer of the present invention may include conventional leuco dyes. Specific examples of such conventional leuco dyes which are employed alone or in combination include:
- 2-(p-acetylanilino)-6-(N-n-amyl-N-n-butylamino)  
 fluoran,  
 2-benzylamino-6-(N-ethyl-p-toluidino)fluoran,  
 2-benzylamino-6-(N-methyl-2,4-dimethylanilino)fluoran,  
 2-benzylamino-6-(N-ethyl-2,4-dimethylanilino)fluoran,  
 2-dibenzylamino-6-(N-methyl-p-toluidino)fluoran,  
 2-dibenzylamino-6-(N-ethyl-p-toluidino)fluoran,  
 2-(di-p-methylbenzylamino)-6-(N-ethyl-p-toluidino) 50  
 fluoran,  
 2-( $\alpha$ -phenylethylamino)-6-(N-ethyl-p-toluidino)fluoran,  
 2-methylamino-6-(N-methylanilino)fluoran,

17

|                                                                       |    |
|-----------------------------------------------------------------------|----|
| 2-methylamino-6-(N-ethylanilino)fluoran,                              | 5  |
| 2-methylamino-6-(N-propylanilino)fluoran,                             |    |
| 2-ethylamino-6-(N-methyl-p-toluidino)fluoran,                         |    |
| 2-methylamino-6-(N-methyl-2,4-dimethylanilino)fluoran,                | 10 |
| 2-ethylamino-6-(N-ethyl-2,4-dimethylanilino)fluoran,                  | 10 |
| 2-dimethylamino-6-(N-methylanilino)fluoran,                           |    |
| 2-dimethylamino-6-(N-ethylanilino)fluoran,                            |    |
| 2-diethylamino-6-(N-methyl-p-toluidino)fluoran,                       | 15 |
| 2-diethylamino-6-(N-ethyl-p-toluidino)fluoran,                        | 15 |
| 2-dipropylamino-6-(N-methylanilino)fluoran,                           |    |
| 2-dipropylamino-6-(N-ethylanilino)fluoran,                            |    |
| 2-amino-6-(N-methylanilino)fluoran,                                   | 20 |
| 2-amino-6-(N-ethylanilino)fluoran,                                    | 20 |
| 2-amino-6-(N-propylanilino)fluoran,                                   |    |
| 2-amino-6-(N-methyl-p-toluidino)fluoran,                              |    |
| 2-amino-6-(N-ethyl-p-toluidino)fluoran,                               | 25 |
| 2-amino-6-(N-propyl-p-toluidino)fluoran,                              | 25 |
| 2-amino-6-(N-methyl-p-ethylanilino)fluoran,                           |    |
| 2-amino-6-(N-ethyl-p-ethylanilino)fluoran,                            |    |
| 2-amino-6-(N-propyl-p-ethylanilino)fluoran,                           | 30 |
| 2-amino-6-(N-methyl-2,4-dimethylanilino)fluoran,                      | 30 |
| 2-amino-6-(N-ethyl-2,4-dimethylanilino)fluoran,                       |    |
| 2-amino-6-(N-propyl-2,4-dimethylanilino)fluoran,                      |    |
| 2-amino-6-(N-methyl-p-chloroanilino)fluoran,                          | 35 |
| 2-amino-6-(N-ethyl-p-chloroanilino)fluoran,                           | 35 |
| 2-amino-6-(N-propyl-p-chloroanilino)fluoran,                          |    |
| 1,2-benzo-6-(N-ethyl-N-isoamylamino)fluoran,                          |    |
| 1,2-benzo-6-dibutylaminofluoran,                                      |    |
| 1,2-benzo-6-(N-ethyl-N-cyclohexylamino)fluoran,                       | 40 |
| 1,2-benzo-6-(N-ethyl-p-toluidino)fluoran,                             |    |
| 2-anilino-3-methyl-6-(N-2-ethoxypropyl-N-ethylamino)fluoran,          |    |
| 2-(p-chloroanilino)-6-(N-n-octylamino)fluoran,                        | 45 |
| 2-(p-chloroanilino)-6-(N-n-palmitylamino)fluoran,                     |    |
| 2-(p-chloroanilino)-6-(di-n-octylamino)fluoran,                       |    |
| 2-benzoylamino-6-(N-ethyl-p-toluidino)fluoran,                        |    |
| 2-(o-methoxybenzoylamino)-6-(N-methyl-p-toluidino)fluoran,            | 50 |
| 2-dibenzylamino-4-methyl-6-diethylaminofluoran,                       |    |
| 2-dibenzylamino-4-methoxy-6-(N-methyl-p-toluidino)fluoran,            |    |
| 2-dibenzylamino-4-methyl-6-(N-ethyl-p-toluidino)fluoran,              | 55 |
| 2-( $\alpha$ -phenylethylamino)-4-methyl-6-diethylaminofluoran,       |    |
| 2-(p-toluidino)-3-(t-butyl)-6-(N-methyl-p-toluidino)fluoran,          | 60 |
| 2-(o-methoxycarbonylanilino)-6-diethylaminofluoran,                   |    |
| 2-acetylamino-6-(N-methyl-p-toluidino)fluoran,                        |    |
| 4-methoxy-6-(N-ethyl-p-toluidino)fluoran,                             |    |
| 2-ethoxyethylamino-3-chloro-6-dibutylaminofluoran,                    |    |
| 2-dibenzylamino-4-chloro-6-(N-ethyl-p-toluidino)fluoran,              |    |
| 2-( $\alpha$ -phenylethylamino)-4-chloro-6-diethylaminofluoran,       | 65 |
| 2-(N-benzyl-p-trifluoromethylanilino)-4-chloro-6-diethylaminofluoran, |    |
| 2-anilino-3-methyl-6-pyrrolidinofluoran,                              |    |

18

2-anilino-3-chloro-6-pyrrolidinofluoran,  
2-anilino-3-methyl-6-(N-ethyl-N-tetrahydrofurfurylamo)fluoran,  
2-mesidino-4',5'-benzo-6-diethylaminofluoran,  
2-(m-trifluoromethylanilino)-3-methyl-6-pyrrolidinofluoran,  
2-( $\alpha$ -naphthylamino)-3,4-benzo-4'-bromo-6-(N-benzyl-N-cyclohexylamino)fluoran,  
2-piperidino-6-diethylaminofluoran,  
2-(N-n-propyl-p-trifluoromethylanilino)-6-morpholinofluoran,  
2-(di-N-p-chlorophenyl-methylamino)-6-pyrrolidinofluoran,  
2-(N-n-propyl-m-trifluoromethylanilino)-6-morpholinofluoran,  
1,2-benzo-6-(N-ethyl-N-n-octylamino)fluoran,  
1,2-benzo-6-diallylaminofluoran,  
1,2-benzo-6-(N-ethoxyethyl-N-ethylamino)fluoran, benzoleucomethyleneblue,  
2-[3,6-bis(diethylamino)]-6-(o-chloroanilino)xanthyl benzoic acid lactam,  
2-[3,6-bis(diethylamino)]-9-(o-chloroanilino)xanthyl benzoic acid lactam,  
3,3-bis(p-dimethylaminophenyl)phthalide,  
3,3-bis(p-dimethylaminophenyl)-6-dimethylaminophthalide (i.e., crystal violet lactone)  
3,3-bis(p-dimethylaminophenyl)-6-diethylaminophthalide,  
3,3-bis(p-dimethylaminophenyl)-6-chlorophthalide,  
3,3-bis(p-dibutylaminophenyl)phthalide,  
3-(2-methoxy-4-dimethylaminophenyl)-3-(2-hydroxy-4,5-dichlorophenyl)phthalide,  
3-(2-hydroxy-4-dimethylaminophenyl)-3-(2-methoxy-5-chlorophenyl)phthalide,  
3-(2-hydroxy-4-dimethoxyaminophenyl)-3-(2-methoxy-5-chlorophenyl)phthalide,  
3-(2-hydroxy-4-dimethylaminophenyl)-3-(2-methoxy-5-nitrophenyl)phthalide,  
3-(2-hydroxy-4-diethylaminophenyl)-3-(2-methoxy-5-methylphenyl)phthalide,  
3-(2-methoxy-4-dimethylaminophenyl)-3-(2-hydroxy-4-chloro-5-methoxyphenyl)phthalide,  
3,6-bis(dimethylamino)fluorenespiro(9,3')-6'-dimethylaminophthalide,  
6'-chloro-8'-methoxy-benzoindolino-spiropyran, and  
6'-bromo-2'-methoxy-benzoindolino-spiropyran.

The recording layer of the recording material of the present invention preferably includes phenolic compounds having the following formula (7) as a coloring developer to obtain good preservability and good resistance to light of the recording material:

(7)



wherein X4 represents a divalent group including a hetero atom and f is 0 or 1; R19 represents a divalent hydrocarbon group and g is 0 or 1; X5 represents a divalent group having a hetero atom; R20 represents a hydrocarbon group having from 1 to 22 carbon atoms; p is 0 or an integer of from 1 to 4, and when p is 2 to 4, each of R19 may be the same or different from each other and each of X5 may be the same or different from each other; and q is an integer of from 1 to 3.

In formula (7), R19 and R20 are independently a hydrocarbon group which is optionally substituted with a group such as a hydroxy group, a halogen atom or an alkoxy group and which may be aliphatic hydrocarbon groups, aromatic hydrocarbon groups or hydrocarbon groups having both an aliphatic hydrocarbon group and an aromatic hydrocarbon group. The aliphatic hydrocarbon groups may be linear or branched, and may include an unsaturated bonding. The total carbon number of R19 and R20 is preferably not less than 7, and more preferably not less than 10, to maintain good color formation/erasure properties of the recording material.

Suitable groups for use as R19 include groups shown in Table 9 other than a direct bonding.

TABLE 9



TABLE 9-continued



10 wherein q, q', q'' and q''' are independently an integer.

Suitable groups for use as R20 include groups shown in Table 10.

TABLE 10



35 wherein q, q', q'' and q''' are independently an integer which is not greater than the carbon atoms of R20, and the total carbon number in a group is not greater than the carbon number of R20.

40 Suitable groups for use as X4 and X5 include divalent groups including at least one of groups, —NH—, —CO—, —O—, —S— and —SO<sub>2</sub>—. Specific examples of such groups include groups shown in Table 11.

TABLE 11



TABLE 11-continued



More preferably, the phenolic compounds for use as a <sup>20</sup> coloring developer in the recording layer include compounds shown in Table 12.

TABLE 12



TABLE 12-continued

|                                                                                   |      |
|-----------------------------------------------------------------------------------|------|
|  | (27) |
|-----------------------------------------------------------------------------------|------|

wherein  $r$ ,  $r'$  and  $s$  are independently an integer under the conditions that R19 and R20 are the groups mentioned above, and  $X5'$  and  $X5''$  independently represent one of the groups which are described for use as  $X5$ .

More specifically, specific examples of the compounds having formula (20) include compounds shown in Table 13, but are not limited thereto.

TABLE 13

|                                                                                      |    |
|--------------------------------------------------------------------------------------|----|
|     | 15 |
|    | 20 |
|    | 25 |
|    | 30 |
|  | 35 |
|  | 40 |
|  | 45 |
|  | 50 |
|  | 55 |
|  | 60 |
|  | 65 |

TABLE 13-continued

TABLE 13-continued

|                                                                                                                                                                                         |
|-----------------------------------------------------------------------------------------------------------------------------------------------------------------------------------------|
| HO—  —COO—(CH <sub>2</sub> ) <sub>r</sub> —NHCONH—(CH <sub>2</sub> ) <sub>s-1</sub> CH <sub>3</sub>    |
| HO—  —O—(CH <sub>2</sub> ) <sub>r</sub> —NHCO—(CH <sub>2</sub> ) <sub>s-1</sub> CH <sub>3</sub>        |
| HO—  —O—(CH <sub>2</sub> ) <sub>r</sub> —CONH—(CH <sub>2</sub> ) <sub>s-1</sub> CH <sub>3</sub>        |
| HO—  —O—(CH <sub>2</sub> ) <sub>r</sub> —NHCOCONH—(CH <sub>2</sub> ) <sub>s-1</sub> CH <sub>3</sub>    |
| HO—  —O—(CH <sub>2</sub> ) <sub>r</sub> —CONHNHCO—(CH <sub>2</sub> ) <sub>s-1</sub> CH <sub>3</sub>    |
| HO—  —O—(CH <sub>2</sub> ) <sub>r</sub> —NHCONH—(CH <sub>2</sub> ) <sub>s-1</sub> CH <sub>3</sub>      |
| HO—  —S—(CH <sub>2</sub> ) <sub>r</sub> —NHCO—(CH <sub>2</sub> ) <sub>s-1</sub> CH <sub>3</sub>       |
| HO—  —S—(CH <sub>2</sub> ) <sub>r</sub> —CONH—(CH <sub>2</sub> ) <sub>s-1</sub> CH <sub>3</sub>      |
| HO—  —S—(CH <sub>2</sub> ) <sub>r</sub> —NHCOCONH—(CH <sub>2</sub> ) <sub>s-1</sub> CH <sub>3</sub>  |
| HO—  —S—(CH <sub>2</sub> ) <sub>r</sub> —CONHNHCO—(CH <sub>2</sub> ) <sub>s-1</sub> CH <sub>3</sub>  |
| HO—  —S—(CH <sub>2</sub> ) <sub>r</sub> —NHCONH—(CH <sub>2</sub> ) <sub>s-1</sub> CH <sub>3</sub>    |
| HO—  —CO—(CH <sub>2</sub> ) <sub>r</sub> —NHCO—(CH <sub>2</sub> ) <sub>s-1</sub> CH <sub>3</sub>     |
| HO—  —CO—(CH <sub>2</sub> ) <sub>r</sub> —CONH—(CH <sub>2</sub> ) <sub>s-1</sub> CH <sub>3</sub>     |
| HO—  —CO—(CH <sub>2</sub> ) <sub>r</sub> —NHCOCONH—(CH <sub>2</sub> ) <sub>s-1</sub> CH <sub>3</sub> |

TABLE 13-continued

|                                                                                                                                                                                                   |
|---------------------------------------------------------------------------------------------------------------------------------------------------------------------------------------------------|
| 5 HO—  —CO—(CH <sub>2</sub> ) <sub>r</sub> —CONHNHCO—(CH <sub>2</sub> ) <sub>s-1</sub> CH <sub>3</sub>          |
| 10 HO—  —CO—(CH <sub>2</sub> ) <sub>r</sub> —NHCONH—(CH <sub>2</sub> ) <sub>s-1</sub> CH <sub>3</sub>           |
| 15 HO—  —NHCONH—(CH <sub>2</sub> ) <sub>r</sub> —NHCO—(CH <sub>2</sub> ) <sub>s-1</sub> CH <sub>3</sub>         |
| 20 HO—  —NHCONH—(CH <sub>2</sub> ) <sub>r</sub> —NHCO—(CH <sub>2</sub> ) <sub>s-1</sub> CH <sub>3</sub>         |
| 25 HO—  —NHCONH—(CH <sub>2</sub> ) <sub>r</sub> —CONHNHCO—(CH <sub>2</sub> ) <sub>s-1</sub> CH <sub>3</sub>     |
| 30 HO—  —NHCONH—(CH <sub>2</sub> ) <sub>r</sub> —NHCONH—(CH <sub>2</sub> ) <sub>s-1</sub> CH <sub>3</sub>      |
| 35 HO—  —CONHNHCO—(CH <sub>2</sub> ) <sub>r</sub> —NHCO—(CH <sub>2</sub> ) <sub>s-1</sub> CH <sub>3</sub>     |
| 40 HO—  —CONHNHCO—(CH <sub>2</sub> ) <sub>r</sub> —CONH—(CH <sub>2</sub> ) <sub>s-1</sub> CH <sub>3</sub>     |
| 45 HO—  —CONHNHCO—(CH <sub>2</sub> ) <sub>r</sub> —NHCOCONH—(CH <sub>2</sub> ) <sub>s-1</sub> CH <sub>3</sub> |
| 50 HO—  —CONHNHCO—(CH <sub>2</sub> ) <sub>r</sub> —CONHNHCO—(CH <sub>2</sub> ) <sub>s-1</sub> CH <sub>3</sub> |
| 55 HO—  —CONHNHCO—(CH <sub>2</sub> ) <sub>r</sub> —NHCONH—(CH <sub>2</sub> ) <sub>s-1</sub> CH <sub>3</sub>   |
| 60 HO—  —NHNHCONH—(CH <sub>2</sub> ) <sub>r</sub> —NHCO—(CH <sub>2</sub> ) <sub>s-1</sub> CH <sub>3</sub>     |
| 65 HO—  —NHNHCONH—(CH <sub>2</sub> ) <sub>r</sub> —CONH—(CH <sub>2</sub> ) <sub>s-1</sub> CH <sub>3</sub>     |

TABLE 13-continued

|  |    |
|--|----|
|  | 5  |
|  | 10 |
|  | 15 |
|  | 20 |
|  | 25 |
|  | 30 |
|  | 35 |

Similarly, specific examples of the phenolic compounds having formulas (19), and (21) to (27) include compounds similar to those shown in Table 13, but are not limited thereto.

Even more specifically, specific examples of the phenolic compounds having the following formula shown in Table 13 include compounds shown in Table 14.

TABLE 14

|  |    |
|--|----|
|  | 40 |
|  | 45 |
|  | 50 |
|  | 55 |
|  | 60 |
|  | 65 |
|  |    |
|  |    |

TABLE 14-continued

|  |    |
|--|----|
|  | 5  |
|  | 10 |
|  | 15 |
|  | 20 |
|  | 25 |
|  | 30 |
|  | 35 |
|  | 40 |
|  | 45 |
|  | 50 |
|  | 55 |
|  | 60 |
|  | 65 |
|  |    |

Among these coloring developers, compounds having the following formula (8) are preferable.



wherein X4' represents a divalent group including a hetero atom and f is 0 or 1; X5 represents a divalent group including a hetero atom; R19 represents a divalent hydrocarbon group and g is 0 or 1; R20 represents a hydrocarbon group having from 1 to 22 carbon atoms; p is 0 or an integer of from 1 to 4, and when p is 2 or more, each of R19 may be the same or different from each other and each of X5 may be the same or different from each other; and q is an integer of from 1 to 3.

In the present invention, other compounds can also be employed as a coloring developer in combination with the phenolic compounds mentioned above.

Suitable compounds for use as a coloring developer in combination with the phenolic compounds mentioned above include compounds which have both a structure capable of developing a coloring agent and a structure capable of controlling cohesive force and which are disclosed in Japanese Laid-Open Patent Publication No. 5-124360 in which organic phosphate compounds, carboxylic acid compounds and phenolic compounds each of which has a long chain hydrocarbon group are exemplified as a typical coloring developer. Specific examples of such compounds include: organic phosphates compounds

dodecyl phosphonate, tetradecyl phosphonate, hexadecyl phosphonate, octadecyl phosphonate, eicosyl phosphonate, docosyl phosphonate, tetracosyl phosphonate, ditetradecyl phosphate, dihexadecyl phosphate, dioctadecyl phosphate, dieicosyl phosphate and dibehenyl phosphate; aliphatic carboxylic acid compounds

2-hydroxy tetradecanoic acid, 2-hydroxy hexadecanoic acid, 2-hydroxy octadecanoic acid, 2-hydroxy eicosanoic acid, 2-hydroxy docosanoic acid, 2-bromo hexadecanoic acid, 2-bromo octadecanoic acid, 2-bromo eicosanoic acid, 2-bromo docosanoic acid, 3-bromo octadecanoic acid, 3-bromo docosanoic acid, 2, 3-dibromo octadecanoic acid, 2-fluoro dodecanoic acid, 2-fluoro tetradecanoic acid, 2-fluoro hexadecanoic acid, 2-fluoro octadecanoic acid, 2-fluoro eicosanoic acid, 2-fluoro docosanoic acid, 2-iodo hexadecanoic acid, 2-iodo octadecanoic acid, 3-iodo hexadecanoic acid, 3-iodo octadecanoic acid and perfluoro octadecanoic acid; and aliphatic dicarboxylic acid compounds and aliphatic tricarboxylic acid compounds

2-dodecyloxsuccinic acid, 2-tetradecyloxsuccinic acid, 2-hexadecyloxsuccinic acid, 2-octadecyloxsuccinic acid, 2-eicosyloxsuccinic acid, 2-docosyloxsuccinic acid, 2-dodecylthiosuccinic acid, 2-tetradecylthiosuccinic acid, 2-hexadecylthiosuccinic acid, 2-octadecylthiosuccinic acid, 2-eicosylthiosuccinic acid, 2-docosylthiosuccinic acid, 2-tetracosylthiosuccinic acid, 2-hexadecylthiosuccinic acid, 2-octadecylthiosuccinic acid, 2-eicosylthiosuccinic acid, dodecylsuccinic acid, tetradecylsuccinic acid, pentadecylsuccinic acid, hexadecylsuccinic acid, octadecylsuccinic acid, eicosylsuccinic acid, docosylsuccinic acid, 2,3-dihexadecylsuccinic acid, 2,3-dioctadecylsuccinic acid, 2-methyl-3-hexadecylsuccinic acid, 2-methyl-3-octadecylsuccinic acid, 2-octadecyl-3-hexadecylsuccinic acid, hexadecylmalonic acid, octadecylmalonic acid, eico-

sylmalonic acid, docosylmalonic acid, dihexadecylmalonic acid, dioctadecylmalonic acid, didocosylmalonic acid, methyloctadecylmalonic acid, 2-hexadecylglutaric acid, 2-octadecylglutaric acid, 2-eicosylglutaric acid, docosylglutaric acid, 2-pentadecyladicpic acid, 2-octadecyladicpic acid, 2-eicosyladicpic acid, 2-docosyladicpic acid, 2-hexadecanoyloxy propane-1,2,3-tricarboxylic acid and 2-octadecanoyloxy propane-1,2,3-tricarboxylic acid.

The mixing ratio of the coloring agent and the coloring developer in the recording layer, which depends on the materials of the coloring agent and the coloring developer used, is from about 1/0.1 to about 1/20 by mole, and preferably from about 1/0.2 to about 1/10, to maintain good image density of the recorded image.

The recording layer preferably includes a crosslinked resin to obtain good heat resistance. In addition, the protective layer preferably includes a crosslinked resin to make the recording material resistant to heat of a recording device such as a thermal printhead and to make the recording material and recorded images resistant to chemicals, water, light and rubbing.

A crosslinked resin can be obtained by heating a mixture of a crosslinking agent and a crosslinkable resin having an active group which can react with the crosslinking agent upon application of heat.

Specific examples of such a heat-crosslinkable resin include resins having an active group such as a hydroxy group, a carboxy group and the like, e.g., phenoxy resins, polyvinyl butyral resins, cellulose acetate propionate and cellulose acetate butyrate. In addition, a copolymer of a monomer having an active group such as a hydroxy group, a carboxyl group or the like and a monomer such as vinyl chloride, an acrylic monomer, styrene or the like can be employed. Specific examples of such a copolymer include vinyl chloride-vinyl acetate-vinyl alcohol copolymers, vinyl chloride-vinyl acetate-hydroxypropyl acrylate copolymers, vinyl chloride-vinyl acetate-maleic anhydride copolymers and the like.

Suitable crosslinking agents which can crosslink these resins upon application of heat include isocyanate compounds, amino resins, phenol resins, amines, epoxy compounds and the like. For example, specific examples of such isocyanate compounds include poly isocyanate compounds having a plurality of isocyanate groups such as hexamethylene diisocyanate (HDI), tolylene diisocyanate (TDI), xylylene diisocyanate (XDI), and adducts of these isocyanate compounds with trimethylol propane and the like, baret type compounds of these isocyanate compounds, isocyanurate type compounds of these isocyanate compounds and blocked isocyanate compounds of these isocyanate compounds.

As for the addition quantity of the crosslinking agents, the ratio of the number of active groups included in the resin to the number of functional groups included in the crosslinking agent is preferably from about 0.01 to about 2 to maintain good heat resistance and good image formation/erasure properties of the recording material.

In addition, the recording layer and the protective layer may include a crosslinking promoter, which is a catalyst useful for this kind of reaction, for example, tertiary amines such as 1,4-diaza-bicyclo(2.2.2) octane, and metal compounds such as organic tin compounds.

Crosslinking can be effected by application of an electron beam or ultraviolet light. Suitable monomers useful for forming a crosslinked recording layer and protective layer which can be crosslinked upon application of electron beam or ultraviolet light include, but are not limited to:

## 31

monomers having one functional group

methyl methacrylate, ethyl methacrylate, n-butyl methacrylate, iso-butyl methacrylate, t-butyl methacrylate, 2-ethylhexyl methacrylate, lauryl methacrylate, tridecyl methacrylate, stearyl methacrylate, cyclohexyl methacrylate, benzyl methacrylate, methacrylic acid, 2-hydroxyethyl methacrylate, 2-hydroxypropyl methacrylate, dimethylaminoethyl methacrylate, methyl chloride salts of dimethylaminoethyl methacrylate, diethylaminoethyl methacrylate, glycidyl methacrylate, tetrahydrofurfuryl methacrylate, allyl methacrylate, 2-ethoxyethyl methacrylate, 2-ethylhexyl acrylate, 2-ethoxyethyl acrylate, 2-ethoxyethoxyethyl acrylate, 2-hydroxyethyl acrylate, 2-hydroxypropyl acrylate, dicyclopentenylethyl acrylate, N-vinyl pyrrolidone and vinyl acetate.

monomers having two functional groups

ethylene glycol dimethacrylate, triethylene glycol dimethacrylate, tetraethylene glycol dimethacrylate, 1,3-butylene glycol dimethacrylate, 1,6-hexanediol dimethacrylate, 1,4-butanediol diacrylate, 1,6-hexanediol diacrylate, 1,9-nonanediol diacrylate, neopentyl glycol diacrylate, tetraethylene glycol diacrylate, tripropylene glycol diacrylate, polypropylene glycol diacrylate, diacrylate esters of an adduct of bisphenol A with ethylene oxide, glycerin methacrylate acrylate, diacrylate esters of an adduct of neopentyl glycol with two moles of propylene oxide, diethylene glycol diacrylate, polyethylene glycol (400) diacrylate, diacrylate esters of an ester of hydroxy pivalate and neopentyl glycol, 2,2-bis(4-acryloyloxydiethoxyphenyl)propane, neopentyl glycol diadipate diacrylate, diacrylate esters of an adduct of neopentyl glycol hydroxypivalate with  $\epsilon$ -caprolactone, 2-(2-hydroxy-1,1-dimethyl-ethyl)-5-hydroxymethyl-5-ethyl-1,3-dioxane diacrylate, tricyclodecane dimethylol diacrylate, adducts of tricyclodecane dimethylol diacrylate with  $\epsilon$ -caprolactone, and 1,6-hexanediol glycidyl ether diacrylate.

monomers having three or more functional groups

trimethylol propane trimethacrylate, trimethylol propane triacrylate, acrylate esters of an adduct of glycerin with propylene oxide, trisacryloyloxyethyl phosphate, penterythritol acrylate, triacrylate esters of an adduct of trimethylol propane with three moles of propylene oxide, dipenterythritol polyacrylate, polyacrylate esters of an adduct of dipentaerythritol with  $\epsilon$ -caprolactone, dipentaerythritol propionate triacrylate, triacrylate esters of hydroxypivalic aldehyde modified dimethylol propane, dipentaerythritol propionate tetraacrylate, ditrimethylol propane tetraacrylate, dipentaerythritol propionate pentaacrylate, dipentaerythritol hexaacrylate and adducts of dipentaerythritol hexaacrylate with  $\epsilon$ -caprolactone.

oligomers

adducts of bisphenol A with diepoxy acrylic acid.

When a resin is crosslinked using ultraviolet light, one or more of the following photopolymerization initiators and photopolymerization promoters can be used in the recording layer and the protective layer.

Specific examples of such photopolymerization initiators include:

benzoin ethers such as isobutyl benzoin ether, isopropyl benzoin ether, benzoin ethyl ether and benzoin methyl ether;  $\alpha$ -acyloxime esters such as 1-phenyl-1,2-propanedione-2-(o-ethoxycarbonyl)oxime; benzyl ketals such as 2,2-dimethoxy-2-phenyl acetophenone and benzyl hydroxycyclohexylphenyl ketone; acetophenone derivatives such as diethoxy acetophenone and 2-hydroxy-2-methyl-1-phenylpropane-1-one; and ketones such as benzophenone, 1-chlorothioxanthone, 2-chlorothioxanthone,

## 32

isopropylthioxanthone, 2-methylthioxanthone and 2-chlorobenzophenone. These photopolymerization initiators are employed alone or in combination.

The content of the photopolymerization initiator in the recording layer or the protective layer is preferably from about 0.005 to about 1.0 part by weight, and more preferably from about 0.01 to about 0.5 part by weight, per 1 part by weight of the monomer or the oligomer.

Suitable photopolymerization promoters include aromatic tertiary amines and aliphatic amines. Specific examples of such photopolymerization promoters which are employed alone or in combination include p-dimethylamino benzoic acid isoamyl ester, p-dimethylamino benzoic acid ethyl ester and the like. The content of the photopolymerization promoter in the recording layer or the protective layer is preferably from about 0.1 to about 5 parts by weight, and more preferably from about 0.3 to about 3 parts by weight, per 1 part by weight of the photopolymerization initiator.

Suitable light sources useful for irradiating ultraviolet light include mercury-vapor lamps, metal-halide lamps, gallium lamps, mercury-xenon lamps, flashing lamps and the like. The light source should be selected so that the spectrum of the ultraviolet light irradiated from the light source corresponds to the absorption spectrum of the photopolymerization initiator and the photopolymerization promoter included in the protective layer. Irradiation conditions of ultraviolet light such as output of lamp power, irradiation width and feeding speed (i.e., irradiation time) should be determined so that the resin in the recording layer or the protective layer can be securely crosslinked.

Electron beam irradiation apparatus includes scanning type and non-scanning type electron beam irradiation apparatus which is selected depending on the irradiation area and the irradiation dose required for crosslinking the recording layer or the protective layer. Irradiation conditions such as electron beam current, irradiation width and irradiation speed should be determined depending on the irradiation dose required for crosslinking the resin included in the recording layer or the protective layer.

The recording layer of the recording material of the present invention is a layer in which a coloring agent and a coloring developer are included in a crosslinked resin. More preferably, the coloring agent and the coloring developer are finely and uniformly dispersed in the crosslinked resin. Even more preferably, the coloring agent and the coloring developer are dispersed while they form complex particles. These complex particles can be obtained, for example, by melting (or dissolving in a solvent) a mixture of a coloring agent and a coloring developer and then cooling the mixture (or drying the solvent). The recording layer including the complex particles can be obtained by coating on a substrate a recording layer coating liquid in which each of a coloring agent and a coloring developer is dispersed or dissolved in a respective solvent and then mixed, or both of them are dispersed or dissolved in a solvent, and then drying the coated liquid. The coloring agent and the coloring developer may be used while being microencapsulated. The recording layer can be crosslinked by a heat crosslinking method, an ultraviolet light crosslinking method or an electron beam crosslinking method. Crosslinking conditions depend on the material of the crosslinkable resin used in the recording layer. For example, the recording layer can be crosslinked upon application of high temperature heat for a short time or can be crosslinked upon application of low temperature heat for a long time. The recording layer can also be crosslinked by the ultraviolet light crosslinking method or the electron beam crosslinking method.

The weight ratio of the total of the coloring agent and the coloring developer to the resin in the recording layer is preferably from about 0.1/1 to about 10/1 to maintain good heat resistance of the recording layer and good image density of the recorded image.

The recording layer of the recording material of the present invention may include auxiliary agents such as dispersants, surfactants, electroconductive agents, fillers, lubricants, antioxidants, photostabilizers, ultraviolet light absorbing agents, color formation stabilizers, and color erasure promoters.

The recording layer may include a thermoplastic resin together with the crosslinked resin. Specific examples of such a thermoplastic resin include polyvinyl chloride resins, polyvinyl acetate resins, vinyl chloride-vinyl acetate copolymers, polystyrene resins, styrene copolymers, phenoxy resins, polyester resins, aromatic polyester resins, polyurethane resins, polycarbonate resins, polyacrylate resins, polymethacrylate resins, acrylic copolymers and maleic anhydride copolymers.

The recording material of the present invention may include a protective layer formed on the recording layer. The protective layer preferably includes a crosslinked resin which is crosslinked upon application of heat, ultraviolet light, electron beam, or the like. By using such a crosslinked resin in the protective layer, the recording material has good ability to be used with thermal printheads and good durability even when the recording material is used repeatedly.

Suitable resins for use in the protective layer include the crosslinked resins which are described for use in the recording layer.

The protective layer may include a resin other than the crosslinked resin. Specific examples of such a resin include polyvinyl alcohol resins, styrene-maleic anhydride copolymers, carboxyl modified polyethylene resins, melamine-formaldehyde resins and urea-formaldehyde resins.

The protective layer may include auxiliary agents such as electroconductive agents which are described for use in the recording layer, stick-preventing agents such as cationic polymers, silicone resins, fluorine-containing resins, phosphate compounds and polyoxyethylene compounds, fillers and lubricants which improve the feeding properties and the wearing resistance of the recording material and which prevent the recording material from sticking to a thermal printhead, ultraviolet absorbing agents and the like.

The recording material of the present invention may include an adhesive layer, an intermediate layer, an under-coat layer, a back-coat layer and a magnetic recording layer other than the recording layer and the protective layer formed on the recording layer. These layers may be colored or non-colored. The magnetic recording layer may be formed on the side of a substrate on which the recording layer is formed or on the opposite side of the substrate.

An intermediate layer is preferably formed between the recording layer and the protective layer to obtain good adhesion thereof and to prevent the recording layer from deteriorating, which is caused by the coating operation of the protective layer and the migration of a component included in the protective layer. The intermediate layer and the protective layer preferably have relatively low oxygen transmittance to obtain good light resistance of the recorded image by preventing the coloring agent and the coloring developer from oxidizing caused by contacting with oxygen.

The recording material may include an under-coat layer between the substrate and the recording layer to effectively utilize heat applied for recording images, to obtain good

adhesion between the recording layer and the substrate and/or to prevent the substrate from deteriorating caused by contacting with the recording layer coating liquid. The heat insulating under-coat layer can be formed by coating a coating liquid in which hollow particles are dispersed in a resin solution.

Suitable resins for use in the intermediate layer or the under-coat layer include resins which are described for use in the recording layer. In addition, the recording layer, the protective layer, the intermediate layer and the under-coat layer may include an inorganic or an organic filler such as calcium carbonate, magnesium carbonate, titanium dioxide, silica, aluminum hydroxide, kaolin, talc and the like. Further, these layers may include lubricants, surfactants and the like.

A suitable substrate for use in the recording material of the present invention includes any substrate which can support the recording layer, such as paper, resin films, synthetic paper, metal foils, glass plates or complex substrates thereof.

20 The substrate may be non-colored or colored and may be transparent or opaque. The substrate may be a complex substrate in which two or more substrates are combined. Suitable thickness of the substrate is from a few  $\mu\text{m}$  to a few mm.

25 The recording material of the present invention may be adhered to a supporting material with an adhesive layer. The adhesive layer may be formed on a part of the recording material or on the entire recording material. The recording material which is adhered to a supporting material may be laminated with films or the like.

The recording material of the present invention can be processed into any shape such as sheet, card, roll and the like.

30 The reversible thermosensitive recording material of the present invention may include an irreversible thermosensitive recording layer. The color of the image of the irreversible thermosensitive recording layer may be the same as or different from that of the reversible thermosensitive recording layer. The irreversible thermosensitive recording layer is preferably formed under the reversible thermosensitive recording layer and the coloring temperature of the irreversible thermosensitive recording layer is preferably higher than that of the reversible thermosensitive recording layer.

35 In addition, the recording material of the present invention may have a print layer thereon. The print layer can be formed, for example, by offset printing, gravure printing, ink jet printing, thermal transfer printing, sublimation thermal transfer printing or the like. Further, the print layer and the recording material having the print layer may be covered entirely or partially by a protective layer (an overprint layer, i.e., an OP layer) which includes a crosslinked resin.

40 Images can be recorded in the recording material of the present invention by heating the recording material, for example, with a thermal pen, a thermal printhead, laser or the like, at an image forming temperature for a short time. When the heating is stopped, the applied heat is quickly diffused, namely, the recorded image is quickly cooled; thereby a stable image can be formed in the recording material. The recorded image can be erased by heating the recording layer at a temperature not lower than the image forming temperature  $T_1$  with an appropriate heating device and then gradually cooling the recording layer, or by heating the recording layer at a temperature in an image erasing temperature range, i.e., a temperature not lower than the image erasing temperature  $T_2$  but lower than the image forming temperature  $T_1$ . The latter image erasing method is preferable because images can be rapidly erased. In addition,

35

the recorded image can be also erased by heating a wide area of the recording layer or heating the recording layer for a long time and then cooling the recording layer. This is because in each case the recording layer is gradually cooled. Suitable heating devices useful for erasing images include heaters such as a ceramic heater, a plane heater, a heat bar, a heat roller or heat stamp; hot air blowing devices; or thermal printheads. When a thermal printhead is used for erasing images, the heat energy applied to the recording layer is preferably controlled so as to be relatively low compared to the heat energy for image recording by controlling the applied voltage and/or pulse width of a pulse applied to the thermal printhead. By using this method, the image recording and erasing operations can be performed with only one thermal printhead, which allows the so-called "overwriting". Needless to say, images can be erased by heating the recording layer at a temperature in an image erasing temperature range with a heater such as ceramic heaters, plane heaters, heat bars, heat rollers or heat stamps.

Having generally described this invention, a further understanding can be obtained by reference to certain specific examples which are provided herein for purposes of illustration only and are not intended to be limiting. In the descriptions in the following examples, numbers represent weight ratios in parts, unless otherwise specified.

## EXAMPLES

### Example 1

#### (Formation of recording layer)

A mixture of the following compounds was pulverized and dispersed in a ball mill in order that the average particle diameter of the solid components in the liquid was from 1 to 4  $\mu\text{m}$ , thus a liquid A was prepared:

#### (Formulation of liquid A)

2-anilino-3-methyl-6-dibutylaminofluoran (coloring agent) 2  
Coloring developer having the following formula



Color formation/erasure controlling agent having the following formula  
 $\text{CH}_3(\text{CH}_2)_4-\text{NHCONH}-(\text{CH}_2)_7\text{CH}_3$   
15% acryl polyol resin solution 120  
(solvent: tetrahydrofuran)

Ten (10) parts of adduct type hexamethylene diisocyanate (Colonate HL, manufactured by Nippon Polyurethane Industry Co., Ltd., ethyl acetate solution having a solid content of 75%) were mixed to the liquid A and the mixture was stirred to prepare a recording layer coating liquid.

The recording layer coating liquid was coated with a wire bar on a substrate of a polyethylene terephthalate (PET) film having a thickness of 180  $\mu\text{m}$ , dried at 100° C. for 3 minutes, and then heated at 60° C. for 24 hours to form a recording layer of about 8.0  $\mu\text{m}$  in a dry thickness.

36

#### (Formation of protective layer)

The following compounds were mixed to prepare a protective layer coating liquid:

5

#### (Formulation of protective layer coating liquid)

|                                                                   |    |
|-------------------------------------------------------------------|----|
| Urethane acrylate type resin crosslinkable with ultraviolet light | 10 |
| (C7-157, manufactured by Dainippon Ink and Chemicals Inc.)        | 90 |
| Ethyl acetate                                                     |    |

The thus prepared protective layer coating liquid was coated on the previously prepared recording layer with a wire bar, dried and then fed under an ultraviolet light radiation lamp, whose irradiation power was 80 W/cm, at a feeding speed of 9 m/min to obtain a crosslinked protective layer having a thickness of 3  $\mu\text{m}$ .

20 Thus, a reversible thermosensitive recording material of the present invention was obtained.

#### (Image recording method)

An image was recorded in each of three sheets of the recording material using a thermal recording apparatus, manufactured by Ohkura Electric Co., Ltd., under the conditions that the voltage applied to a thermal printhead was 13.3 v and the pulse width was 1.2 ms. The image density of the recorded image which was measured with Macbeth reflection densitometer RD914 was 1.13. The recorded image formed in one of the sheets was then erased by heating at 110° C. for 0.5 seconds using a heat gradient tester manufactured by Toyo Seiki Co., Ltd. to erase the image. The residual image density of the recording material after the image was erased was 0.03. The recording material remained in a good state without deformation of the recording material even after the above-mentioned recording/erasing operation was repeated 50 times.

35 40 The image density retention of the recording material was 90% after the image formed in another sheet was preserved in a dry place at 50° C. for 24 hours.

In addition, in order to measure a residual image density after light irradiation, the procedure for image formation and erasure mentioned above was performed using the other sheet of the recording material after the image was exposed to light, which was radiated by a fluorescent lamp and whose illuminance was 5500 lux, for 100 hours. The residual image density after light irradiation was 0.03, and even when these image forming and erasing operations were repeated, there occurred no problem such as misunderstanding of image information in the recording material.

45 50 55 This reversible thermosensitive recording material had such good image formation/erasure properties, good durability, good preservability and good light resistance that the recording material could be stably used for a long time even when applied for practical use.

### Example 2

The procedure for preparation of the recording material in Example 1 was repeated except that the coloring developer and the color formation/erasure controlling agent were replaced with the following coloring developer and the following color formation/erasure controlling agent, respectively:

Coloring developer



Color formation/erasure controlling agent



The procedure for evaluation of the recording material in Example 1 was repeated.

The image density of the recorded image was 1.12. The residual image density of the recording material after the image was erased under the same conditions as mentioned above was 0.02. The recording material remained in a good state without deformation of the recording material even after the above-mentioned recording/erasing operation was repeated 50 times. In addition, the image density retention was 92% and the residual image density after light irradiation was 0.03, and there occurred no problem such as misunderstanding of image information in the recording material even when the image recording/erasing operations were repeated.

This reversible thermosensitive recording material had such good image formation/erasure properties, good durability, good preservability and good light resistance that the recording material could be stably used for a long time even when applied for practical use.

### Example 3

The procedure for preparation of the recording material in Example 2 was repeated except that the color formation/erasure controlling agent was replaced with the following color formation/erasure controlling agent:

Color formation/erasure controlling agent



The procedure for evaluation of the recording material in Example 1 was repeated.

The image density of the recorded image was 1.10. The residual image density was 0.02. The recording material remained in a good state without deformation of the recording material even after the above-mentioned recording/erasing operation was repeated 50 times. In addition, the image density retention was 65% and the residual image density after light irradiation was 0.02, and there occurred no problem such as misunderstanding of image information in the recording material even when the image recording/erasing operations were repeated.

This reversible thermosensitive recording material had such good image formation/erasure properties, good durability, good preservability and good light resistance that the recording material could be stably used for a long time even when applied for practical use.

### Example 4

The procedure for preparation of the recording material in Example 2 was repeated except that the coloring agent was replaced with 3-(4-diethylamino-2-ethoxyphenyl)-3-N-ethyl-2-methylindole-3-yl)-4-azaphthalide and the color formation/erasure controlling agent was replaced with the following color formation/erasure controlling agent:

Color formation/erasure controlling agent



The procedure for evaluation of the recording material in Example 1 was repeated.

The image density of the recorded image was 0.89. The residual image density was 0.01. The recording material remained in a good state without deformation of the recording material even after the above-mentioned recording/erasing operation was repeated 50 times. In addition, the image density retention was 75% and the residual image density after light irradiation was 0.01, and there occurred no problem such as misunderstanding of image information in the recording material even when the image recording/erasing operations were repeated.

This reversible thermosensitive recording material had such good image formation/erasure properties, good durability, good preservability and good light resistance that the recording material could be stably used for a long time even when applied for practical use.

### Example 5

The procedure for preparation of the recording material in Example 4 was repeated except that the color formation/erasure controlling agent was replaced with the following color formation/erasure controlling agent:

Color formation/erasure controlling agent



The procedure for evaluation of the recording material in Example 1 was repeated.

The image density of the recorded image was 0.88. The residual image density was 0.02. The recording material remained in a good state without deformation of the recording material even after the above-mentioned recording/erasing operation was repeated 50 times. In addition, the image density retention was 88% and the residual image density after light irradiation was 0.02, and there occurred no problem such as misunderstanding of image information in the recording material even when the image recording/erasing operations were repeated.

This reversible thermosensitive recording material had such good image formation/erasure properties, good durability, good preservability and good light resistance that the recording material could be stably used for a long time even when applied for practical use.

### Example 6

The procedure for preparation of the recording material in Example 4 was repeated except that the color formation/erasure controlling agent was replaced with the following color formation/erasure controlling agent:

Color formation/erasure controlling agent



The procedure for evaluation of the recording material in Example 1 was repeated.

The image density of the recorded image was 0.88. The residual image density was 0.01. The recording material remained in a good state without deformation of the recording material even after the above-mentioned recording/erasing operation was repeated 50 times. In addition, the image density retention was 85% and the residual image density after light irradiation was 0.02, and there occurred no problem such as misunderstanding of image information in the recording material even when the image recording/erasing operations were repeated.

This reversible thermosensitive recording material had such good image formation/erasure properties, good

39

durability, good preservability and good light resistance that the recording material could be stably used for a long time even when applied for practical use.

## Example 7

The procedure for preparation of the recording material in Example 2 was repeated except that the coloring agent was replaced with 3,3-bis(2-ethoxy-4-diethylaminophenyl)-4-azaphthalide and the color formation/erasure controlling agent was replaced with the following color formation/erasure controlling agent:

Color formation/erasure controlling agent



The procedure for evaluation of the recording material in Example 1 was repeated.

The image density of the recorded image was 0.82. The residual image density was 0.02. The recording material remained in a good state without deformation of the recording material even after the above-mentioned recording/erasing operation was repeated 50 times. In addition, the image density retention was 82% and the residual image density after light irradiation was 0.02, and there occurred no problem such as misunderstanding of image information in the recording material even when the image recording/erasing operations were repeated.

This reversible thermosensitive recording material had such good image formation/erasure properties, good durability, good preservability and good light resistance that the recording material could be stably used for a long time even when applied for practical use.

## Example 8

The procedure for preparation of the recording material in Example 2 was repeated except that the color formation/erasure controlling agent was replaced with the following color formation/erasure controlling agent:

Color formation/erasure controlling agent



The procedure for evaluation of the recording material in Example 1 was repeated.

The image density of the recorded image was 1.10. The residual image density was 0.02. The recording material remained in a good state without deformation of the recording material even after the above-mentioned recording/erasing operation was repeated 50 times. In addition, the image density retention was 95% and the residual image density after light irradiation was 0.03, and there occurred no problem such as misunderstanding of image information in the recording material even when the image recording/erasing operations were repeated.

This reversible thermosensitive recording material had such good image formation/erasure properties, good durability, good preservability and good light resistance that the recording material could be stably used for a long time even when applied for practical use.

## Comparative Example 1

The procedure for preparation of the recording material in Example 1 was repeated except that the color formation/erasure controlling agent was eliminated from the recording layer coating liquid and the coloring developer was replaced with the following coloring developer:

6,090,748  
40

Coloring developer



The procedure for evaluation of the recording material in Example 1 was repeated.

The image density of the recorded image was 1.08. The residual image density was 0.03. The recording material remained in a good state without deformation of the recording material even after the above-mentioned recording/erasing operation was repeated 50 times. In addition, the image density retention was 38% and the residual image density after light irradiation was 0.04.

This comparative recording material had relatively low image retention compared to the recording materials of the present invention and therefore image contrast was gradually decreased when repeatedly applied for practical use.

## Comparative Example 2

The procedure for preparation of the recording material in Example 1 was repeated except that the color formation/erasure controlling agent was eliminated from the recording layer coating liquid and the coloring developer was replaced with the following coloring developer:

Coloring developer



The procedure for evaluation of the recording material in Example 1 was repeated.

The image density of the recorded image was 1.12. The residual image density was 0.20. The recording material remained in a good state without deformation of the recording material even after the above-mentioned recording/erasing operation was repeated 50 times. In addition, the image density retention was 79% and the residual image density after light irradiation was 0.25.

This comparative recording material had relatively high residual image density compared to the recording materials of the present invention because the former images were not clearly erased. Therefore recorded images could not be easily recognized because the former images and the current images were overlapped.

As can be understood from the detailed description of the reversible thermosensitive recording material of the present invention, the reversible thermosensitive recording material of the present invention has good preservability, quick erasability, good durability and good image forming/erasing properties without generating deformation.

Additional modifications and variations of the present invention are possible in light of the above teachings. It is therefore to be understood that within the scope of the appended claims the invention may be practiced other than as specifically described herein.

This application is based on Japanese Patent Applications Nos. 09-185917 and 09-185918, both filed on Jun. 26, 1997, the entire contents of which are herein incorporated by reference.

What is claimed is:

1. A reversible thermosensitive recording material comprising a recording layer which is formed overlying at least one side of a substrate and which comprises an electron donating coloring agent and an electron accepting coloring developer,

wherein the recording layer achieves a colored state when heated at a temperature not lower than an image forming temperature and then cooled at a cooling speed (a), and the recording layer in the colored state achieves a non-colored state when heated at a temperature lower than the image forming temperature and not lower than an image erasing temperature, or when heated at a temperature not lower than the image forming temperature and then cooled relatively slowly compared to the cooling speed (a),

and wherein the recording layer further comprises at least one color formation/erasure controlling agent having a formula selected from the group consisting of the following formulas (1) and (2):



wherein  $X_1$  represents a group selected from the group consisting of moieties in Table 3;  $X_2$  represents a divalent group selected from the group consisting of moieties in Table 4;  $R_1$  represents a divalent hydrocarbon group having from 2 to 20 carbon atoms, and when  $X_1$  is a carboxyl group, the  $R_1$  group adjacent to  $X_1$  is a linear hydrocarbon group having not less than 7 carbon atoms;  $R_2$  represents a hydrocarbon group having from 1 to 22 carbon atoms; and  $n$  is an integer of from 1 to 4, and when  $n$  is 2 or more, each of  $R_1$  may be the same or different from each other and each of  $X_2$  may be the same or different from each other; and



wherein  $Y_1$  and  $Y_2$  are independently selected from the group consisting of moieties in Table 4;  $R_1$  represents a divalent hydrocarbon group having from 2 to 20 carbon atoms;  $R_2$  and  $R_2'$  independently represent a hydrocarbon group having from 1 to 22 carbon atoms; and  $n$  is 0 or an integer of from 1 to 4, and when  $n$  is 2 or more, each of  $R_1$  may be the same or different from each other and each of  $Y_2$  may be the same or different from each other.

2. The reversible thermosensitive recording material according to claim 1, wherein said at least one color formation/erasure controlling agent comprises a compound of formula (1).

3. The reversible thermosensitive recording material according to claim 1, wherein said at least one color formation/erasure controlling agent comprises a compound of formula (2).

4. The reversible thermosensitive recording material according to claim 1, wherein the electron donating coloring agent comprises a fluoran compound having the following formula (3):



15 wherein  $R_3$  and  $R_4$  independently represent a lower alkyl group, an aryl group, a substituted aryl group or a hydrogen atom, and  $R_3$  and  $R_4$  may combine with each other to form a ring;  $R_5$  represents a lower alkyl group, a halogen atom or a hydrogen atom; and  $R_6$  represents a lower alkyl group, a halogen atom, a hydrogen atom or a substituted anilino group having the following formula (4):



30 wherein  $R_7$  represents a lower alkyl group or a hydrogen atom;  $X_3$  represents a lower alkyl group or a halogen atom; and  $b$  is 0 or an integer of from 1 to 3.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 99



(6)

5

10

wherein R13, R14, R15 and R16 independently represent a lower alkyl group or a hydrogen atom; and R17 and R18 independently represent an alkyl group, an alkoxy group or a hydrogen atom.

7. The reversible thermosensitive recording material according to claim 1, wherein the electron accepting coloring developer comprises a phenolic compound having the following formula (7):

(7)



25

wherein X4 represents a divalent group having a hetero atom and f is 0 or 1; X5 represents a divalent group having a hetero atom; R19 represents a divalent hydrocarbon group and g is 0 or 1; R20 represents a hydrocarbon group having from 1 to 22 carbon atoms; p is 0 or an integer of from 1 to 4, and when p is 2 or more, each of R19 may be the same or different from each other and each of X5 may be the same or different from each other; and q is an integer of from 1 to 3.

8. The reversible thermosensitive recording material according to claim 1, wherein the recording layer further comprises a crosslinked resin.

9. The reversible thermosensitive recording material according to claim 1, wherein the recording material further comprises a protective layer which is formed overlying the recording layer and which comprises a crosslinked resin.

10. The reversible thermosensitive recording material according to claim 1, wherein the recording material is card shaped or sheet shaped.

11. The reversible thermosensitive recording material according to claim 1, wherein the recording material comprises a print layer which is formed overlying at least one side of the substrate.

12. The reversible thermosensitive recording material according to claim 1, wherein the recording material has an image density retention not less than about 60% when the recording material having an image of the colored state is allowed to settle in a dry place at 50° C. for 24 hours, a residual image density not greater than about 0.03 when the recording material having an image of the colored state is heated at 110° C. for 0.5 seconds to erase the image, and a residual image density after light irradiation not greater than about 0.04 when the recording material having an image of the colored state is heated at 110° C. for 0.5 seconds to erase the image after light of 5,000 lux is irradiated to the recording material for 100 hours.

13. The reversible thermosensitive recording material according to claim 1, wherein the electron accepting coloring developer has a long chain alkyl group in which the total number of carbon atoms is not less than 8.

14. A reversible thermosensitive recording method comprising the steps of:

preparing a reversible thermosensitive recording material which comprises a substrate, a recording layer which is formed overlying at least one side of the substrate and which comprises an electron donating coloring agent and an electron accepting coloring developer, said recording material optionally further comprising any one or more of a protective layer which is formed overlying the recording layer, a magnetic recording layer and a print layer, wherein the recording layer achieves a colored state when heated at a temperature not lower than an image forming temperature and then cooled at a cooling speed (a), and the recording layer in the colored state achieves a non-colored state when heated at a temperature lower than the image forming temperature or when heated at a temperature not lower than the image forming temperature and then cooled relatively slowly compared to the cooling speed (a), and wherein the recording layer further comprises at least one color formation/erasure controlling agent having a formula selected from the group consisting of the following formulas (1) and (2):



wherein X1 represents a group selected from the group consisting of moieties in Table 3; X2 represents a divalent group selected from the group consisting of moieties in Table 4; R1 represents a divalent hydrocarbon group having from 2 to 20 carbon atoms, and when X1 is a carboxyl group, the R1 group adjacent to X1 is a linear hydrocarbon group having not less than 7 carbon atoms; R2 represents a hydrocarbon group having from 1 to 22 carbon atoms; and n is an integer of from 1 to 4, and when n is 2 or more, each of R1 may be the same or different from each other and each of X2 may be the same or different from each other; and



wherein Y1 and Y2 are independently selected from the group consisting of moieties in Table 4; R1 represents a divalent hydrocarbon group having from 2 to 20 carbon atoms; R2 and R2' independently represent a hydrocarbon group having from 1 to 22 carbon atoms; and n is 0 or an integer of from 1 to 4, and when n is 2 or more, each of R1 may be the same or different from each other and each of Y2 may be the same or different from each other;

imagewise heating the recording layer at a temperature not lower than the image forming temperature and then cooling the recording layer at the cooling speed (a) to form a colored image in the recording layer; and heating the recording layer at a temperature lower than the image forming temperature and not lower than the image erasing temperature to erase the image.

15. A reversible thermosensitive recording apparatus comprising:

an image forming device which imagewise heats a recording layer of a reversible thermosensitive recording material at a temperature not lower than an image forming temperature to form a colored image, wherein the recording material comprises an electron donating coloring agent and an electron accepting coloring developer in the recording layer and optionally further comprises any one or more of a protective layer, a magnetic layer and a print layer, and wherein the

**45**

recording layer achieves a colored state when heated at a temperature not lower than the image forming temperature and then cooled at a cooling speed (a), and the recording layer in the colored state achieves a non-colored state when heated at a temperature lower than the image forming temperature and not lower than an image erasing temperature or when heated at a temperature not lower than the image forming temperature and then cooled relatively slowly compared to the cooling speed (a), and wherein the recording layer further comprises at least one color formation/erasure controlling agent having a formula selected from the group consisting of the following formulas (1) and (2):



wherein X1 represents a group selected from the group consisting of moieties in Table 3; X2 represents a divalent group selected from the group consisting of moieties in Table 4; R1 represents a divalent hydrocarbon group having from 2 to 20 carbon atoms, and when X1 is a carboxyl group, the R1 group adjacent to X1 is a linear hydrocarbon group having not less than 7 carbon atoms; R2 represents a

10

20

**46**

hydrocarbon group having from 1 to 22 carbon atoms; and n is an integer of from 1 to 4, and when n is 2 or more, each of R1 may be the same or different from each other and each of X2 may be the same or different from each other; and



wherein Y1 and Y2 are independently selected from the group consisting of moieties in Table 4; R1 represents a divalent hydrocarbon group having from 2 to 20 carbon atoms; R2 and R2' independently represent a hydrocarbon group having from 1 to 22 carbon atoms; and n is 0 or an integer of from 1 to 4, and when n is 2 or more, each of R1 may be the same or different from each other and each of Y2 may be the same or different from each other; and

an image erasing device which heats the recording layer at a temperature lower than the image forming temperature and not lower than the image erasing temperature to erase the colored image, wherein the erasing device is one of a ceramic heater, a plane heater, a heat roller, a heat bar and a thermal printhead.

\* \* \* \* \*